# EUROPEAN PATENT SPECIFICATION

(11) **EP 0 998 544 B1**
(45) Date of publication and mention of the grant of the patent: **02.07.2003**
(21) Application number: 98945164.6
(22) Date of filing: 23.07.1998
(51) Int. Cl.: C10M 169/06, C10N 30/06

(54) **GREASE COMPOSITION FOR A CONSTANT VELOCITY JOINT**
SCHMIERFETTZUSAMMENSETZUNG FÜR HOMOKINETISCHE KUPPLUNG
COMPOSITION GRAISSEUSE POUR JOINT HOMOCINETIQUE

(30) Priority: 24.07.1997 JP 21417197
(43) Date of publication of application: 10.05.2000
(73) Proprietor: SHELL INTERNATIONALE RESEARCH MAATSCHAPPIJ B.V., 2596 HR Den Haag (NL)
(72) Inventor: OZAKI, Takahiro, Minato-ku, Tokyo 135 (JP); MUNAKATA, Tomoo, Minato-ku, Tokyo 135 (JP); YOSHIDA, Tsutomu, Minato-ku, Tokyo 135 (JP); MASUMORI, Ryuichi, Minato-ku, Tokyo 135 (JP)
(86) International application number: EP9804983
(87) International publication number: WO99005240

(56) References cited:
- EP-A- 0 617 117
- US-A- 3 505 223
- US-A- 4 923 625
- US-A- 4 986 923

## Description

The present invention relates to the use of grease compositions in a constant velocity joint also referred to as CVJ. Grease lubrication of CVJ's is extremely harsh since it is carried out under conditions of friction under high surface pressures where slipping and rolling over in reciprocating movement are intermixed. The present invention relates to the use of a grease composition for lubricating a constant velocity joint having an extremely long-lived durability and to prevent the occurrence of abnormal wear and flaking.

CVJ's in automobiles are employed in front-wheel drive vehicles and four-wheel drive vehicles, as well as rear-wheel drive vehicles, and demand tends to increase. As automobiles achieve higher speeds, higher outputs and lighter weights, CVJ's become smaller, whilst sustaining higher torques and being applied at higher speeds. Therefore, the grease must meet increasing performance specifications. CVJ's can be categorised as fixed joint or plunging joint depending on the mechanism. Conditions are extremely harsh for fixed joints since these are generally used for wheels and are employed at high angles and under high surface pressure.

Usually, CVJ greases contain lithium soap as thickener and additives such as sulphur/phosphorus-based extreme pressure agents and molybdenum disulphide. Recently, urea-based greases containing various extreme pressure agents have become more common. These have outstanding heat-resisting properties.

JP-A (Japanese Laid-Open Patent Application) H 6-57284 (1994) discloses a grease composition for a constant velocity joint in which a urea grease contains, as essential constituents, (A) a molybdenum dialkyldithiocarbamide sulphide, (B) an extreme pressure additive comprising a specific zinc dithiophosphate compound, and (C) an epoxy-modified aliphatic acid ester or an epoxy-modified aliphatic acid glyceride.

Further urea greases have been described in JP-B (Examined Japanese Patent Document) H 4-34590 (1992), JP-A H 6-57283 (1994), JP-A H 6-100878 (1994), JP-A H 7-197072 (1995) and JP-A H 8-41485 (1996), and US-A-4,840,740, US-A-5,160,645 and US-A-5,449,471. These documents teach to add an organic molybdenum compound to a base grease together with yet other additives (such as zinc dithiophosphate) to reduce frictional wear and, as a result, prevent flaking.

However, these compositions still suffer from flaking which stems from metal surface fatigue caused by roll-over slipping friction in complex reciprocating movements of tne inner and outer wheel channels and balls as well as cages and balls in a CVJ mechanism.

In US-A-4,923,625 grease compositions are described for use in cutting and grinding operations. The compositions contain a mixture of a metal thiosulfate and a metal phosphate to impart both extreme pressure and antiwear properties to a base lubricant.

US-A-3,505,223 describes a lubricating composition comprising a major amount of an organic liquid lubricating oil or grease and an extreme pressure reducing amount of a metal thiosulphate.

CVJ-producing manufacturers and grease-supplying manufacturers are trying to predict flaking in CVJ with the help of frictional wear tests such as the four-ball EP tests described in ASTM D2596. Where durability in CVJ's is concerned appropriate greases cannot be selected using the test apparatuses mentioned above.
This is thought to be due to the complexity of the lubrication conditions. Therefore, the performance in terms of the flaking life, state of wear and the like is evaluated using a bench test apparatus in which an actual CVJ is used.

The fact that substances which exhibit outstanding results in general frictional wear tests do not necessarily prevent CVJ flaking or have long durability, makes it difficult to develop CVJ flaking prevention technology.

The aim of the present invention is to provide a constant velocity joint grease composition whereby CVJ flaking can be prevented.

The present invention further relates to the use of a grease composition for lubricating a constant velocity joint, which grease composition comprises base oil and urea-based thickener, which composition further contains from 0.05 to 30% by weight of metal thiosulphate, based on weight of base oil and urea-based thickener.

The base oil used in the present embodiment can be a mineral oil or a synthetic oil such as an ester oil, ether oil or hydrocarbon oil, or an oil mixed from these. Preferably, the base oil is a mineral oil.

Any urea-based thickener can be used. Examples of urea-based thickeners include diurea, triurea and tetraurea. Further, it is also possible to use various thickeners containing urea compounds such as urea-urethane compounds and urea-imido compounds.

The metal thiosulphate used in the present invention, can contain any metal that is capable of forming a metal thiosulphate salt. Typical examples are lithium, sodium, potassium, manganese, calcium, barium, strontium, titanium, zirconium, cadmium, zinc, nickel, cobalt, copper, iron, magnesium, lead, tin, silver, or a mixture of these.

A useful class of metal thiosulphate is represented by the following formula where R represents a hydrocarbon radical containing 1 to 30 carbon atoms, M is a metal capable of forming a metal thiosulphate salt and n is the valence of M. Examples of this class of metal thiosulphates are sodium ethyl thiosulphate, potassium benzyl thiosulphate and barium isoamyl thiosulphate. The compounds can be prepared by reacting an alkyl halide with sodium thiosulphate.

Preferably, the metal thiosulphate used in the present invention is sodium thiosulphate. Most preferably, the sodium thiosulphate is Na₂S₂O₃ (anhydrous), Na₂S₂O₃.5H₂O (pentahydrate) or a mixture of these. Further, it is possible to use commercial additives containing sodium thiosulphate, such as "Desilube 88," (trade mark) Desilube Technology, Inc. USA.

The amount of sodium thiosulphate added is from 0.05 to 30 percent by weight, and preferably from 0.2 to 20 percent by weight based on weight of base oil and urea-based thickener, more preferably 0.2 to 10% by weight, more preferably 0.2 to 8% by weight, most preferably 0.5 to 6% by weight. If the amount is less than 0.05 percent by weight, the flaking-preventing effect is insufficient. If the amount is more than 30 percent by weight, there is no further increase in the effect.

The composition of the present invention can further contain one or more known additives such as phenol-based and amine-based antioxidants, organic molybdenum compounds, molybdenum disulphide, sulphur-modified fats and oils, sulphur-modified olefins, zinc dithiophosphate, thiophosphate, phosphite, phosphate, and polysulphide, and other such extreme pressure/anti-wear agents, polybutenes, polymethacrylates and other such viscosity enhancers.

Greases according to the invention and comparative examples were obtained using the formulations shown in Table 1 and Table 2 by adding the additives to a base grease and processing in a three-roll mill. The compositions of the base greases are given below. The base oil was purified mineral oil with a viscosity at 100°C of 15mm²/S.

### I. Diurea grease

A grease was obtained by reacting diphenylmethane-4,4'-diisocyanate (295.2 g) and octylamine (304.8g) in a base oil (5,400 g), and uniformly dispersing the resulting urea compound. The urea compound content was 10 percent by weight.

### II. Tetraurea grease

A grease was obtained by reacting diphenylmethane-4,4'-diisocyanate (334.2 g), stearylamine (345.6 g) and ethylenediamine (40.2 g) in a base oil (5,280 g), and uniformly dispersing the resulting urea compound. The urea compound content was 12 percent by weight.

### III. Lithium soap grease

A grease was obtained by dissolving lithium 12-hydroxystearate (540 g) in a base oil (5,460 g), and uniformly dispersing. The lithium soap content was 9 percent by weight.

The resulting greases were subjected to durability testing on mounts using actual CVJ's, and the degree of flaking was checked.

### Test conditions

| | |
|---|---|
| Rotational speed | 1,400 rpm |
| Load torque | 294 N m |
| Joint angle | 6 deg |
| Joint type | Burfield joint |

Further, the fusion load (N) was determined using the four-ball EP test specified in ASTM D2596. The results are collated in Tables 1 to 4.

It should be noted that, in the tables, *1 to 7 and ** are as follows.
*1 "Desilube 88" (trade mark, made by Desilube Technology Inc.) is an inorganic additive containing sodium thiosulphate.
*2 "Moliban A" (trade mark, made by the Vanderbilt company) is molybdenum dithiocarbamate.
*3 "Sakura Lube 600" (trade mark, made by Asahi Denka) is molybdenum dithiocarbanate.
*4 "Sakura Lube 300" (trade mark, made by Asahi Denka) is molybdenum dithiophosphate.
*5 "Lubrizol 1395" (trade mark, made by the Lubrizol company) is zinc dithiophosphate.
*6 "Anguramoru 33" (trade mark, made by the Lubrizol company) is a sulphur-modified olefin.
*7 Iruga Lube TPPT" (trade mark, made by the Ciba-Geigy company) is triphenylphosphorothionate.
**For the degree of flaking, the condition after 12,600,000 revolutions, and the condition after 25,200,000 revolutions of the CVJ was observed and evaluated as follows.
◇ No flaking
o Minor flaking
Δ Moderate flaking
x Extensive flaking

**TABLE 1**

| Embodiment | | | 1 | 2 | 3 | 4 |
|---|---|---|---|---|---|---|
| Composition wt% | Base grease | Diurea grease | 97 | 95 | | 97 |
| | | Tetraurea grease | | | 95 | |
| | Additives | Na₂S₂O₃ (anhydrous) | 3 | 5 | 5 | |
| | | Na₂S₂O₃.5H₂O | | | | 3 |
| | | "Desilube 88" *1 | | | | |
| | Total | | 100 | 100 | 100 | 100 |
| Test results | Four-ball EP test | Fusion load (N) | 6076 | 7840 | 7840 | 6076 |
| | Degree of flaking ** | By 12,600,000 revolutions | ◇ | ◇ | ◇ | o |
| | | By 25,200,000 revolutions | o | ◇ | ◇ | Δ |

**TABLE 2**

| Embodiment | | | 5 | 6 | 7 | 8 |
|---|---|---|---|---|---|---|
| Composition wt% | Base grease | Diurea grease | | 97 | | 99 |
| | | Tetraurea grease | 97 | | 97 | |
| | Additives | Na₂S₂O₃ (anhydrous) | | | | |
| | | Na₂S₂O₃.5H₂O "Desilube 88" *1 | 3 | | | |
| | | | | 3 | 3 | 1 |
| | Total | | 100 | 100 | 100 | 100 |
| Test results | Four-ball EP test | Fusion load (N) | 6076 | >7840 | 7840 | 6076 |
| | Degree of flaking ** | By 12,600,000 revolutions | o | ◇ | ◇ | o |
| | | By 25,200,000 revolutions | Δ | ◇ | ◇ | Δ |

**TABLE 3**

| Embodiment | | | 1 | 2 | 3 | 4 |
|---|---|---|---|---|---|---|
| Composition wt% | Base grease | Diurea grease | | | | 93 |
| | | | | | | |
| | | Tetraurea grease | | | | |
| | | Lithium grease | 97 | 97 | 97 | |
| | Additives | Na₂S₂O₃ (anhydrous) | 3 | | | |
| | | Na₂S₂O₃ 5H₂O | | 3 | | |
| | | "Desilube 88" *1 | | | 3 | |
| | | "Moliban A" *2 | | | | 3 |
| | | "Sakura Lube 600" *3 | | | | |
| | | "Sakura Lube 300" *4 | | | | 2 |
| | | "Lubrizol 1395" *5 | | | | |
| | | "Anguramoru 33" *6 | | | | 1 |
| | | "Icuga Lube TPPT" *7 | | | | |
| | | Molybdenum disulphide | | | | |
| | Total | | 100 | 100 | 100 | 100 |
| | | | | | | |
| Test results | Four-ball EP Fusion load (N) test | | 6076 | 3920 | 6076 | 3087 |
| | Degree of flaking ** | By 12,600,000 revolutions | x | Δ | Δ | x |
| | | By 25,200,000 revolutions | - | x | Δ | - |

As is clear from the results shown in Tables 1 to 4, the grease composition for a constant velocity joint of the present invention has outstanding extreme pressure properties, and provides more effective flaking prevention properties than do conventional greases. This effect improves the durability of constant velocity joints.

## Claims

1. Use of a grease composition for lubricating a constant velocity joint, which grease composition comprises base oil, metal thiosulphate and thickener, **characterised in that** the thickener is a urea-based thickener and that the composition further contains from 0.05 to 30% by weight of metal thiosulphate, based on weight of base oil and urea-based thickener.

2. Use of a grease composition according to claim 1, in which the grease composition contains from 0.2 to 20% by weight of metal thiosulphate.

3. Use of a grease composition according to claim 1 or 2, in which the base oil is a mineral oil.

4. Use of a grease composition according to any one of claims 1 to 3, in which grease composition the metal thiosulphate is sodium thiosulphate.

5. Use of a grease composition according to any one of claims 1 to 4, in which grease composition the urea-based thickener is selected from diurea, triurea and tetraurea.

## Patentansprüche

1. Verwendung einer Schmierfettzusammensetzung zum Schmieren eines homokinetischen Gelenkes, welche Schmierfettzusammensetzung ein Grundöl, Metallthiosulfat und ein Verdickungsmittel umfaßt, **dadurch gekennzeichnet, daß** das Verdickungsmittel ein Verdickungsmittel auf Harnstoffbasis ist und daß die Zusammensetzung weiterhin 0,05 bis 30 Gew.-% Metallthiosulfat, bezogen auf das Gewicht des Grundöls und des Verdickungsmittels auf Harnstoffbasis, enthält.

2. Verwendung einer Schmierfettzusammensetzung nach Anspruch 1, worin die Schmierfettzusammensetzung 0,2 bis 20 Gew.-% Metallthiosulfat enthält.

3. Verwendung einer Schmierfettzusammensetzung nach Anspruch 1 oder 2, worin das Grundöl ein Mineralöl ist.

4. Verwendung einer Schmierfettzusammensetzung nach einem der Ansprüche 1 bis 3, in welcher Schmierfettzusammensetzung das Metallthiosulfat Natriumthiosulfat ist.

5. Verwendung einer Schmierfettzusammensetzung nach einem der Ansprüche 1 bis 4, in welcher Schmierfettzusammensetzung das Verdickungsmittel auf Harnstoffbasis unter Diharnstoff, Triharnstoff und Tetraharnstoff ausgewählt ist.

## Revendications

1. Utilisation d'une composition de graisse pour lubrifier un joint homocinétique, laquelle composition de graisse comprend une huile de base, un thiosulfate métallique et un épaississant, **caractérisée en ce que** l'épaississant est un épaississant à base d'urée et que la composition contient de plus de 0,05 à 30% en poids de thiosulfate métallique, par rapport au poids d'huile de base et d'épaississant à base d'urée.

2. Utilisation d'une composition de graisse suivant la revendication 1, dans laquelle la composition de graisse contient de 0,2 à 20% en poids de thiosulfate métallique.

3. Utilisation d'une composition de graisse suivant l'une ou l'autre des revendications 1 et 2, dans laquelle l'huile de base est une huile minérale.

4. Utilisation d'une composition de graisse suivant l'une quelconque des revendications 1 à 3, composition de graisse dans laquelle le thiosulfate métallique est du thiosulfate de sodium.

5. Utilisation d'une composition de graisse suivant l'une quelconque des revendications 1 à 4, composition de graisse dans laquelle l'épaississant à base d'urée est choisi parmi la diurée, la triurée et la tétraurée.
